

# United States Patent

[11] 3,617,326

[72] Inventors **John R. Zuber**  
Piscataway;  
**Herbert Foxman, Raritan, both of N.J.**  
[21] Appl. No. **802,675**  
[22] Filed **Feb. 26, 1969**  
[45] Patented **Nov. 2, 1971**  
[73] Assignee **RCA Corporation**

[56]

## References Cited

### UNITED STATES PATENTS

|           |         |              |         |
|-----------|---------|--------------|---------|
| 3,320,195 | 5/1967  | Braun.....   | 260/564 |
| 3,294,718 | 12/1966 | Antonen..... | 260/18  |

*Primary Examiner*—Alfred L. Leavitt  
*Assistant Examiner*—M. F. Esposito  
*Attorney*—Glenn H. Bruestle

[54] **METHOD OF BRANDING SILICON PLASTIC SURFACE**

3 Claims, No Drawings

[52] **U.S. Cl.**..... **117/12,**  
117/8, 117/38, 117/47 R, 117/138.8 B, 260/564 A  
[51] **Int. Cl.**..... **B41m 1/30,**  
B44d 1/092  
[50] **Field of Search**..... 117/12, 47  
R, 8, 38, 138.8 B; 260/564 A

**ABSTRACT:** A method of branding the surface of a silicone plastic body so as to improve the adherence of printed trademark and type number indicia on said surface is described. The method comprises treating the surface of the silicone plastic body with a solution consisting of 1,1,3,3, tetramethylguanidine and a surfactant dissolved in an organic solvent. Conveniently, a bibulous material is saturated with the solution, and a silicone plastic body is positioned thereon so that the surface of the body to be branded is in contact therewith. After a few minutes, the silicone plastic body is removed, any excess solution remaining on the body surface is wiped off, and the desired indicia are then printed on the treated surface.

## METHOD OF BRANDING SILICON PLASTIC SURFACE

## BACKGROUND OF THE INVENTION

This invention relates to improved methods of branding the surface of silicone plastic bodies.

Silicone plastics are widely used in the form of sheets, rods and tubes. They are also used to package many types of semiconductor devices, including both discrete units such as diodes or transistors or thyristors, and also integrated circuits. The identification of sheets, rods and tubes of silicone plastic by the brand or trademark of the manufacturer is useful, but is not critical. However, when a wide variety of the different types of semiconductor devices are supplied in a similar package consisting of a silicone plastic, it is imperative that the different type numbers which identify the devices should be clearly and permanently marked on the surface of the plastic package. It has been found that when the surface of a conventional silicone plastic body, such as the silicone plastic package of a semiconductor device, is marked with brand name and type number indicia in the conventional manner by printing on the surface of the silicone plastic package, the numbers and brand names tend to rub off the smooth inert surface of the plastic when the packaged device is handled.

The printed indicia on silicone plastic bodies also become unreadable when they come in contact with various common solvents such as alcohol, acetone, trichlorethylene, detergent solutions, and the like. It then becomes difficult for the user to determine the identity or particular type of each such plastic packaged semiconductor device.

## SUMMARY OF THE INVENTION

The surface of a silicone plastic body is treated with a solution consisting of 1,1,3,3, tetramethylguanidine and a surfactant dissolved in an organic solvent, and the excess solution is removed from the body surface. Desired indicia which are subsequently printed on the treated surface of the plastic body adhere firmly thereto, and are not removed by rubbing, or by dipping in conventional solvents.

## THE PREFERRED EMBODIMENTS

Silicone plastics or resins are high molecular weight polymers characterized by having a long chain composed of alternating atoms of silicon and oxygen, with various organic constituents bonded to the silicon atoms. The typical formula for a silicone resin is  $[R_1R_2SiO]_n$ . The two organic groups or constituents  $R_1$  and  $R_2$  attached to the silicon atom may be different from each other, or may be the same alkyl radical. Silicone resins have properties which make them useful for the packaging of semiconductor devices. These resins are inert, resistant to water and oxidation, stable at temperatures as high as 300° C., and have good dielectric properties.

A surfactant is a substance which even in small amount is capable of producing marked changes in the surface energy of liquid or solid surfaces. Surfactants which are added to a liquid are also known as wetting agents, and tend to lower the surface tension of any system which includes an interface between a liquid phase and another phase. Surfactants have been broadly divided into three types. The first type is the anionic type, which includes compounds having carboxylate groups, and derivatives of sulfuric acid or sulfonic acid. The second type is the cationic type, which generally consists of nitrogen compounds, such as the salts of primary or secondary or tertiary amines. The third type is the nonionic type, and includes polyethylene glycol, polyvinyl alcohol, polyethers, polyesters, and polyhalides. A large variety of surfactants are commercially available, many of them being identified by trade names rather than by composition.

The term "organic solvent" generally refers to an organic compound which is a liquid at room temperature, and is capable of dissolving some organic substances. Organic solvents commercially available include hundreds of simple or complex alcohols, amines, esters, ethers, hydrocarbons, and ketones. Both straight chain and branched chain compounds

are utilized as organic solvents. Also utilized are cyclic compounds such as benzene, toluene, xylene, and cyclohexanol; petroleum fractions such as petrolic ether and kerosene and naphtha; and aliphatic hydrocarbons such as pentane, hexane and heptane. Certain organic solvents such as  $C_4H_9(OC_2H_5)_2OH$ ,  $C_2H_5(OC_2H_5)_2OCOCH_3$ , and  $CH_3OC_2H_4OH$  are generally identified by trade names.

The compound 1,1,3,3, trimethylguanidine is a water-white liquid which boils at about 165° C., and has a molecular weight of 115.18, corresponding to the molecular formula  $C_8H_{15}N$ . The structural formula of this compound may be written as  $(CH_3)_2NC(NH)N(CH_3)_2$ .

## EXAMPLE I

15 A solution is prepared consisting of about 30 milliliters 1,1,2,2, trimethylguanidine in about 70 milliliters of an organic solvent, which in this example is xylene. About 1 or 2 milliliters of a surfactant, which in this example consists of 20 polyethylene glycol, is added to the solution. The precise composition of the solution is not critical, and may range from about 5 to 50 volume percent of 1,1,3,3, trimethylguanidine.

A bibulous material such as a paper towel or blotting paper or cotton cloth or the like is saturated with the solution. This 25 silicone plastic article to be branded, which may for example be an integrated circuit that has been encapsulated in a rectangular mass of the resin, is positioned on the saturated bibulous material so that the surface of the article to be branded is in contact with the saturated bibulous material. 30 After a few minutes, the silicone plastic article is removed. Any excess solution remaining on the surface of the article is wiped off, or is removed by any convenient method, such as by spinning the article, or by directing a stream of dry air against the treated surface.

35 The desired indicia, such as trademark and type numbers, are then printed on the treated surface of the silicone plastic article in the conventional manner. When a silicone plastic article is branded in this manner, it is found that the printed indicia do not rub off easily, and are resistant to the action of 40 common solvents.

An unexpected advantage of this method is that the silicone 45 plastic articles which have been treated as described do not require prompt branding with the desired indicia. After the silicone plastic articles have been treated by the method of this invention, they may be stored for an indefinite period of time before they are branded. It appears that the treatment described changes the nature of the surface of the silicone plastic article in a manner which is either irreversible, or of very long duration.

## EXAMPLE II

In the previous example, a nonionic surfactant was utilized. In the example, the solution consists of about 5 to 50 volume percent 1,1,3,3, trimethylguanidine, the balance being one of the organic solvents previously mentioned. About 1 or 2 milliliters of one of the anionic surfactants is added for each 100 milliliters of the solution. A surface of a silicone plastic article is then treated as described in example I prior to branding this surface by printing the desired indicia thereon.

## EXAMPLE III

In this example, the solution consists of about 5 to 50 volume percent 1,1,3,3, trimethylguanidine, the balance being one of the organic solvents previously mentioned. About 1 to 65 2 milliliters of one of the cationic surfactants is added for each 100 milliliters of the solution. A surface of a silicone plastic article is then treated as described in example I prior to branding this surface by printing the desired indicia thereon. 7

We claim:

1. The method of branding the surface of a silicone plastic body, comprising the steps of treating said surface with a solution consisting of 5 to 50 volume percent of 1,1,3,3, tetramethylguanidine and a surfactant dissolved in an organic solvent;

removing the excess solution from said surface;  
and printing indicia on said treated surface.

2. The method as in claim 1, wherein said silicone plastic body is treated with said solution at room temperature.

3. The method of branding the surface of a silicone plastic article, comprising the steps of preparing a solution consisting of 5 to 50 volume percent of 1,1,3,3, trimethylguanidine and a surfactant dissolved in an organic solvent;

saturating a bibulous material with said solution;

positioning a silicone plastic article on said bibulous material so that the surface of the article to be branded is in contact with the bibulous material for a few minutes;  
removing said article from said bibulous material;  
removing from said surface of said article any of said solution remaining thereon;  
and printing indicia on said treated surface of said silicone plastic article.

\* \* \* \* \*